

May 3, 1949.

W. W. DURFEE, ET AL

2,468,738

METHOD OF BLOWING IN BLAST FURNACES

Filed Jan. 15, 1947

2 Sheets-Sheet 1

*Fig. 1.*



*Fig. 3.*



Walter W. Durfee and <sup>Inventor</sup>  
John P. Foley  
Donald G. Dalton  
Their Attorney

May 3, 1949.

W. W. DURFEE ET AL

2,468,738

METHOD OF BLOWING IN BLAST FURNACES

Filed Jan. 15, 1947

2 Sheets-Sheet 2

*Fig. 2.*



3 Inventor  
Walter W. Durfee and  
John P. Foley  
Donald G. Dalton  
Their Attorney

## UNITED STATES PATENT OFFICE

2,468,738

## METHOD OF BLOWING IN BLAST FURNACES

Walter W. Durfee and John P. Foley, Lorain, Ohio,  
assignors to National Tube Company, a corporation of New Jersey

Application January 15, 1947, Serial No. 722,174

4 Claims. (Cl. 75—41)

1

The present invention relates to blast furnace operation and particularly to an improved method for blowing in a blast furnace.

Among the objects of the invention is the provision of an improved method for blowing in a blast furnace, characterized by ease of operation and a reduction of the time necessary to bring the furnace into operation. The method displays particular advantages when employed in blowing in a banked blast furnace.

Because of fluctuating iron demands, the need for repairs to the furnaces, and other enforced shutdown of the furnace, it is at times necessary to blow in furnaces which have been either live banked or dead banked. In dead banking a blast furnace, the air blast is replaced by a blast relatively free of oxygen, for example, by blast furnace gas or by gas rich in carbon dioxide, nitrogen, or the like, that quickly extinguishes the fire. In the live banking of blast furnaces, some hours before the last cast is made a coke blank is formed in the upper portion of the furnace by charging only coke thereinto. Alternatively, a burden richer in coke than normal can be charged at such time. In live banking, the tuyères and blow pipe are sealed off and the stack effect is relied upon to maintain diminished combustion which is sufficient to prevent extinguishing of the fire.

In the prior methods of blowing in a blast furnace which has been either dead or live banked, it has been customary to light especially prepared and easily ignitable portions of the burden, following which the furnace has been blown in with a blast of air or with oxygen enriched air, admitted through the tuyères. Such methods have not been altogether successful because by their use, even after long periods of blowing, it has been difficult to obtain free running iron in the tap hole or iron notch. It was therefore necessary to employ oxygen lances and other means to cut out the chilled iron at the iron notch and melt it sufficiently to bring about its flow. Such operations at the iron notch are hazardous to the operators, who are exposed to the heat and flames thrown back from the solid iron by the oxygen lances, as well as to the sudden flow of hot iron when a break through occurs. Usually such supplementary heating of the iron notch, with previous methods of blowing in, have to be repeated many times before a good flow of iron is obtained and the furnace blown in with normal blast.

Briefly, the method of the present invention comprises lighting the coke in the vicinity of the iron notch of a dead or live banked furnace in

2

any known manner, and thereafter blowing air into the tap hole or iron notch of the furnace under a pressure sufficient to prevent a flow of iron out of the furnace and for a period long enough to heat up the bottom and hearth uniformly and to melt the residual iron found therein. Before making the first tap of iron from the furnace and following an extended period of such blowing in, a blast of air may be admitted, if desired, through the tuyères to heat up the bosh and stack and bring about a further melting of the iron which now flows easily through the heated hearth, gradually becoming more highly heated and building up a pool or reservoir of molten iron in the bottom.

The blast to be employed through the tap hole may be cold air, hot air, oxygen enriched air, and may even in some cases be undiluted oxygen. The time interval between lighting the furnace and making the first tap obviously depends on many factors, such as the amount of residual iron in the hearth, the net volume of blast admitted through the tap hole, the nature and volume of blast admitted through the tuyères, and the accumulated volume of iron and cinder in the furnace. A blast similar to that admitted to the tap hole can be used in the cinder notch. However, this ordinarily is not necessary for difficulty in iron flow at the cinder notch is rarely experienced.

The invention will be more readily understood by reference to the accompanying drawings in which:

Figure 1 is a schematic view in vertical cross section through a portion of a banked blast furnace in the vicinity of the tuyères and iron notch;

Figure 2 is a similar view of such furnace equipped with the blowing in apparatus of our invention after the furnace has been operated in accordance with our method; and

Figure 3 is a view of a portion of the apparatus employed in practicing the method, the view being taken along the line III—III in Figure 2.

The blast furnace 2, shown schematically in Figures 1 and 2, is provided with a bustle pipe 4 which extends around the furnace carrying the hot blast through the tuyère stocks 8 which are tapped thereinto and thence to the tuyères 6, of which one is shown. The furnace is also provided with an iron notch 9 which is customarily plugged as with clay, not shown, when the furnace is in the banked condition indicated in Figure 1. The contents of the furnace when it is in such banked condition consist of a burden 10, which is a mixture of coke, limestone, and iron

ore. In Figures 1 and 2 the lumps of coke are indicated by the large shapes designated 12, the lumps of iron ore are designated by the small rounded hatched shapes denoted 14, and the lumps of limestone are shown as triangular shapes 16. In the banked condition, whether dead or live, all or substantially all combustion in the vicinity of the hearth below the level of the iron notch 9 has ceased and the residual iron in the hearth solidifies after a time into a solid mass 18.

Blowing in of the furnace shown in Figure 1 in accordance with the invention may conveniently be effected by the use of the apparatus shown connected thereto in Figure 2. Such apparatus consists of the pipe 20 having a valve 22 therein tapped into the tuyère stock 8, as shown, to lead a portion of the blast gas into the iron notch. Pipe 20 is connected to a vertical pipe 26 through the elbow 24 and thence through a series of double elbow connections to the pipe 42 which is inserted into the iron notch 9 after the clay plug has been removed therefrom. Such double elbow connections, which are shown at 30, 34, and 40 between the pipes 26 and 32, 32 and 36, and 36 and 42, respectively, allow a relative freedom of axial movement of pipe 42 so that it may be inserted in the iron notch and withdrawn therefrom while remaining connected to the source of blast. Chain 56, which is shown attached at the elbow joint 40, allows the quick withdrawal of pipe 42 from the iron notch by means such as a winch, not shown, when the flow of iron begins at the notch. The described supplementary blowing means for the iron notch is equipped with a pressure gauge, as at 28, and with an inlet pipe 38 tapped thereinto, pipe 38 being provided with a valve and being connected to a source of oxygen, not shown, to allow the enrichment of the blast with oxygen as desired.

The following specific example, which is illustrative only, demonstrates one manner in which the method of the invention may be carried out. In this instance, the furnace to be blown in had been live banked for about sixty days. The supplementary iron notch blowing apparatus shown in Figure 2 was connected to a tuyère stock in the manner indicated, all tuyères were clayed up, and the peep sights were opened. A hot blast enriched with oxygen was thereupon admitted through the iron notch through pipe 42 and was continued for five hours. The initial static pressure of such blast was about two pounds per square inch, the estimated average volume of hot blast blown through the iron notch through the iron notch blowing apparatus, in which all pipes were four inch size, was 3,000 cubic feet per minute. The enriching oxygen was supplied through pipe 38 at the rate of 350 cubic feet per minute. The temperature of the hot blast in the bustle pipe was 1100° F., the temperature of such blast as it entered the iron notch being estimated at 600° F. After the initial five-hour period, three tuyères in the front of the furnace were opened and a total of about 18,000 cubic feet of hot blast per minute blown through them for an additional five-hour period. The hot enriched blast through pipes 20 and so forth into pipe 42 and thence into the iron notch was maintained, the pressure in such pipes building up slowly to about four pounds per square inch during the ten hours of blowing through the iron notch. Within the one-half hour period following the initial blowing through the iron notch and the five hours of combined blowing, the pressure, as indicated by gauge 28, increased rather quickly to about ten

pounds per square inch, indicating the presence of a substantial body of molten iron at the iron notch zone. Thereupon pipe 42 was quickly withdrawn from the iron notch by chain 56 and a quarter ladle of free running iron and slag was immediately obtained from the notch. After claying up the iron notch in the usual manner normal operating blast on all tuyères was provided and normal operation of the blast furnace resumed.

A consideration of Figure 2 will make clearer the manner in which the blowing in method of the present invention operates. As above indicated, one of the initial steps in the blowing in of a banked furnace is the lighting of the unconsumed burden in the vicinity of the iron notch. It will be apparent, therefore, that such lighted burden when acted upon directly by a blast, and particularly by a hot oxygen enriched blast, will relatively quickly raise the burden, portions of the other furnace contents, and parts of the furnace adjacent thereto to a high temperature. Such high temperature zone is indicated in Figure 2 by the dotted outline 54.

In such high temperature zone the metal refining process of the blast furnace is thus resumed in miniature, the iron ore being reduced to iron which descends in the form of molten iron drops 48 onto the hearth, and the molten slag resulting therefrom, shown as drops 50, likewise trickling through the burden onto the hearth. The blast in the iron notch has the further effect of gradually melting the solidified mass 18 of iron in the hearth. As shown in Figure 2, which represents the condition of the furnace after a substantial period of blowing at the iron notch, a pool of molten iron is formed at 46, and an adjacent zone 44 of semi-molten iron. There will, of course, also be present adjacent the notch a layer of molten slag, designated 52, which floats on top of the molten iron.

By blowing in a furnace in accordance with the present invention, it is possible to accomplish such operation with none of the hazards to the workmen or the difficult cleanups of chilled iron heretofore encountered when blowing in a blast furnace. The uniformity of heating at the iron notch accomplished by our invention makes it possible to blow in a furnace from fully banked condition to normal operation in a total time of less than about twelve hours. Although the invention has been described in connection with the blowing in of a banked furnace, it may be employed to advantage in initially blowing in a furnace with a clean burden.

Although we have described and illustrated preferred embodiments of the method of blowing in a blast furnace in accordance with the invention and a preferred embodiment of the apparatus for carrying out such method, it is to be understood that the invention is not confined thereto but that it is defined within the scope of the following claims.

We claim:

1. The method of blowing in a banked blast furnace comprising sealing the tuyères, lighting the burden in the vicinity of the iron notch, blowing a substantial quantity of oxygen containing blast gas through the iron notch for a substantial length of time, thereupon unsealing the tuyères in the vicinity of the iron notch and blowing oxygen-containing blast gas additionally through such tuyères while maintaining the blast through the iron notch, and after a substantial quantity of molten iron has been obtained on the

hearth in the vicinity of the iron notch, unsealing the remainder of the tuyères and resuming normal furnace blast therethrough.

2. The method of blowing in a banked blast furnace comprising sealing the tuyères, lighting the furnace burden in the vicinity of the iron notch, blowing through the iron notch a substantial quantity of hot blast air for a substantial length of time, thereupon unsealing tuyères in the vicinity of the iron notch and blowing a substantial quantity of blast air therethrough while maintaining the blast at the iron notch, continuing such combined blowing operations until a substantial quantity of molten iron is obtained on the hearth, and then unsealing the remainder of tuyères and resuming normal furnace operations by introducing blast air therethrough.

3. The method of blowing in a banked blast furnace comprising sealing the tuyères, lighting the furnace burden in the vicinity of the iron notch, blowing through the iron notch a substantial quantity of hot blast air enriched with an appreciable percentage of oxygen for a substantial length of time, thereupon unsealing tuyères in the vicinity of the iron notch and introducing substantial quantities of hot blast air therethrough, continuing the blast at the iron notch, such combined blowing operations being continued until a substantial quantity of molten iron is obtained on the hearth, discontinuing the iron notch blast, drawing off the molten iron, unsealing the remainder of the tuyères, and resuming normal operation by blowing blast gas through the tuyères.

4. The method of blowing in a banked blast furnace comprising sealing the tuyères, lighting the furnace burden in the vicinity of the iron notch, blowing through the iron notch hot blast air at a rate on the order of 3000 cubic feet per

minute and at an initial static pressure of about two pounds per square inch, the blast air entering the iron notch at a temperature on the order of 600° F. and being enriched by approximately 350 cubic feet per minute of oxygen, continuing such blast at the iron notch for a period on the order of five hours, thereafter opening a relatively small number of tuyères adjacent the iron notch and introducing hot blast air therethrough in a total quantity on the order of 18,000 cubic feet per minute for an additional period on the order of five hours, while maintaining the iron notch blast simultaneously therewith until a substantial quantity of molten iron is obtained on the hearth as indicated by a rise in back pressure of the iron notch blast, thereupon discontinuing such blast, drawing off the molten iron, unsealing the remainder of the tuyères, and resuming the blast through all tuyères to normal furnace operation.

WALTER W. DURFEE.  
JOHN P. FOLEY.

#### REFERENCES CITED

25 The following references are of record in the file of this patent:

#### UNITED STATES PATENTS

| Number       | Name               | Date          |
|--------------|--------------------|---------------|
| 30 1,507,740 | Kirby -----        | Sept. 9, 1924 |
| 1,654,300    | McGee et al. ----- | Dec. 27, 1927 |
| 2,301,973    | Riddle -----       | Nov. 17, 1942 |

#### OTHER REFERENCES

35 Stahl und Eisen, vol. 45, pages 609-614, April 23, 1925.

"Proceedings of the Blast Furnace and Raw Materials Committee" (A. I. M. E.), vol. 1, 1941, pages 59 and 60.